

## UNITED STATES PATENT OFFICE

2,526,948

PROCESS OF TREATING TEXTILES WITH  
HALF-ACID AMIDE DERIVATIVESChester M. Himmel, Bartlesville, Okla., assignor to  
Phillips Petroleum Company, a corporation of  
DelawareNo Drawing. Application October 23, 1945,  
Serial No. 624,103

13 Claims. (CL 117—138.5)

1

This invention relates to a method of treating textile fibers. In one of its more specific aspects, this invention relates to a method of impregnating textile fibers with cyclic imides.

The process of the present invention provides a method of treating textile fibers and fabrics to impart desirable properties thereto. It is well known that textile fibers generally possess some undesirable properties, such as lack of water resistance, vulnerability to attack by insects, and lack of uniformity in the application of dye materials. The present invention provides a method of treating textile fibers whereby undesirable properties inherent in many textiles can be modified or changed. In many applications the cost of treating textile fibers is of paramount importance. An important feature of this invention is that it provides a process of treating textiles which is simple and effective, and one which can be carried out with a minimum of processing cost.

Textile treating agents can be roughly divided into two classes, those that are impregnated directly, and those that are developed within the interstices of the fiber. In general, the latter method usually leaves the fiber in a more acceptable condition due probably to the fact that the reaction is carried out within the fiber. In many cases, it is difficult to carry out the developed type of impregnation since the reactions are sometimes difficult to control at reasonable temperatures and low cost operating conditions. The present invention provides a process whereby a textile treating agent is rendered water soluble for ease in impregnation and is then made permanently water insoluble by a simple washing and heating process. Aqueous solutions are used in the process of the present invention, thereby providing a low cost vehicle for the reaction and eliminating the danger and fire hazard of the usual organic solvents.

An object of this invention is to provide a method for the treatment of textile fibers. Another object is to provide such a method wherein the textile fibers may be impregnated with a cyclic imide. Another object is to provide a method of treating fibers wherein certain desirable properties may be imparted thereto. Another object of this invention is to provide a process for treating textile fibers to impart desirable properties thereto wherein water is used as the vehicle for the treating agent. Still another object is to provide by the method of this invention an improved textile fiber.

The process of the present invention provides a method of treating textile fibers by developing

2

within the fiber a water-insoluble cyclic imide which is not removed by normal laundering and other water washing. Cyclic imides may be used in accordance with my invention as dye leveling agents, water repelling agents, mothproofing agents, or flame resisting agents for imparting various desirable properties to the fabrics. Other uses will occur to those skilled in the art.

I have found that improved physical properties 10 may be imparted to textile fibers and fabrics by treatment in accordance with the method herein disclosed. These improved properties are the direct result of a process wherein a normally water soluble compound is developed within the fiber 15 and changed to a normally water insoluble compound which has the property of imparting to the treated fiber the characteristic desired. The process is concerned with a method whereby a water soluble intermediate compound can be impregnated in a fiber and converted to a water insoluble cyclic imide by the simple process of 20 washing and heating to temperatures below the decomposition point of the fabric being treated. The cyclic imides which are useful in the present 25 invention are those having five or six members in the imide ring. The compounds which are particularly useful are the cyclic imides produced by the dehydration of a half-acid amide of a dibasic acid selected from the group consisting of maleic, succinic, glutaric, and phthalic acids, their analogues and homologues including the chlorine substituted derivatives of these compounds. In general, the half-acid amide of a dibasic acid capable of forming a cyclic anhydride 30 having from five to six carbon atoms in the ring is useful in the present invention. The half-acid amides useful in the process are, of course, prepared from the selected dibasic acid or its anhydride and a primary amine. The half-acid amides of secondary amines are inoperative in 35 my process.

The half-acid amides of the dibasic acids preferred for use in the present invention are for the most part, water insoluble or difficulty soluble. The water solubility can be increased to a suitable level by the use of alkali, such as sodium or potassium hydroxide or other bases which form soluble salts of the half-acid amide. In accordance with 45 this invention, an alkaline aqueous solution of the half-acid amide of the desired dibasic acid and primary amine is prepared and the fiber is impregnated with this solution. The salt of the half-acid amide thus thoroughly impregnates the fiber. The fiber containing said salt is then contacted with an aqueous solution of a mineral acid,

e. g. hydrochloric acid, which converts said salt to the less soluble half-acid amide. In this step of the process the half-acid amide, which is water insoluble or only slightly water soluble, is developed within the interstices of the fiber. The treated fiber at this stage is not alkali proof or launder proof since a simple alkaline wash would remove much of the impregnant. I have found that the fiber containing the half-acid amide can be made permanently resistant to the effects of laundering by simply heating the fiber containing the half-acid amide to remove water, dehydrating the half-acid amide and forming the cyclic imide corresponding to the half-acid amide which was impregnated within the fiber. The resulting cyclic imide is stable, is water insoluble, and is resistant to laundering. In dye-leveling applications this characteristic of water insolubility is less rigidly adhered to since some developed cyclic imides useful as dye leveling agents are somewhat water soluble. In the process whereby water resistance is imparted to the textile the developed cyclic imide is, of course, highly water insoluble and water resistant.

The reactions involved in carrying out the process of the invention may be illustrated by a specific example in which a half-acid amide of phthalic acid is employed. A half-acid amide of phthalic acid is represented by the structural formula:



where R represents an alkyl, aralkyl or cycloalkyl group. In an alkaline aqueous solution, for example sodium hydroxide, the alkali salt of the half-acid amide is formed:



Upon contacting the impregnated fiber with an aqueous solution of a strong mineral acid, the half-acid amide is again formed as represented by formula I above. Upon dehydration the half-acid amide is converted to the corresponding cyclic imide:



Various imides which may be employed in the process of this invention are useful as dye leveling agents. When the textile fiber or fabric to be dyed is first treated in accordance with the present invention, subsequent dyeing results in evenness of color throughout. Impregnation of fibers with cyclic imides by use of my invention may be employed to render the fibers

flame resistant. The imides which give best results as flameproofing agents are those which contain halogens, particularly those which contain 40 to 60 per cent halogen on a weight basis. These also have good mothproofing qualities. The cyclic imides best suited for waterproofing fabrics are those containing at least sixteen carbon atoms per molecule and preferably more.

The half-acid amide for use in the process of my invention may be made by reacting a primary amine with the desired dibasic acid, or with a suitable derivative thereof such as, for example, the anhydride of the dibasic acid. Halo-substituted acids, acid anhydrides, and the like may be employed, such as, for example, tetrachlorophthalic acid. Primary aliphatic aromatic, and alicyclic amines and halo-substituted derivatives thereof are suitable for use in the preparation of the half-acid amide. The reaction between the anhydride and the primary amine is best carried out in the presence of an inert diluent to control the temperature and viscosity of the reaction mixture. Chloroform and toluene, for example, have been found suitable for use as diluents but other solvents can be used in this preparation. Alternately, the half-acid amide can be prepared by partial hydrolysis of the diamide.

The half-acid amide is converted to the cyclic imide by heating. In general, the process of imide formation takes place at a temperature above about 200° F., the higher molecular weight amides requiring a temperature within the range of 250° F. to 350° F. I have found that the half-acid amides impregnating textile fibers may be converted to the corresponding imides at temperatures below those which cause damage to the fibers which are not melted or decomposed at the temperatures used in the process.

For a fuller understanding of the nature and objects of the invention, reference should be had to the following examples which are given merely to further illustrate the invention and are not to be construed in a limiting sense, all parts given being by weight.

#### EXAMPLE 1

##### *Preparation of N-cyclohexylphthalamic acid*

Phthalic anhydride (74 grams—0.5 mole) was added gradually to a stirred reaction mixture containing cyclohexylamine (99 g.—1.0 mole) in 200 ml. toluene. Reaction occurred spontaneously. The product was washed with dilute hydrochloric acid and then with water. The toluene layer was then extracted with a slight excess of sodium hydroxide. Acidification of the caustic layer gave the free phthalamic acid M. P. 318-319° F. The phthalamic acid loses water at its melting point and forms N-cyclohexylphthalimide.

#### EXAMPLE 2

##### *Preparation of N-dodecylphthalamic acid*

Dodecyl amine (½ mole—92.5 g.) was dissolved in 400 ml. toluene and stirred during the addition of phthalic anhydride (0.5 mole—74 g.). The reaction temperature was held at 160-175° F. during the addition of the phthalic anhydride. The toluene solution was washed several times with large quantities of hot dilute hydrochloric acid to remove excess amine and phthalic acid. Emulsions were broken or controlled by suitable additions of acetone or methanol. The purified phthalic acid was extracted as the sodium salt

and was precipitated from aqueous solution by acidification. The product on drying had M. P. 192° F. and a neutral equivalent of 334 (calc. 333). Heating at 250° F. caused water to be evolved giving the imide, M. P. 147-149° F.

#### EXAMPLE 3

##### *Preparation of N-hexadecyltetrachlorophthalamic acid*

The phthalamic acid from hexadecyl amine and tetrachlorophthalic acid was prepared by the procedure outlined in Example 2. The free phthalamic acid was dissolved in aqueous 10% caustic and used as a textile impregnant.

#### EXAMPLE 4

##### *Waterproofing of cotton textiles*

A 5% solution of N-hexadecyltetrachlorophthalamic acid was prepared in aqueous caustic solution. Cotton squares were impregnated with the solution, squeezed dry and then added to a dilute acid wash containing 10% hydrochloric acid. The cotton was then thoroughly washed with water to remove mineral acid and subsequently dried and heated to 300-350° F. for one to five minutes to cause permanent water repellancy in the fabric.

#### EXAMPLE 5

##### *Chlorinated phthalamic acid*

N-dodecyl phthalamic acid was chlorinated to 50-60% chlorine content by reaction of chlorine on N-dodecyl phthalamic acid in carbon tetrachloride solution. The free acid was used as an impregnant for cotton and wool as outlined in Example 4. The treated textiles were water repellent and moth resistant. The process did not cause an undesirable change in the feel of the fabrics.

#### EXAMPLE 6

##### *Dye leveling agent*

The phthalamic acid from phthalic anhydride and (trihydroxymethyl) methyl amine,  $(\text{CH}_2\text{OH})_3\text{CNH}_2$ , was prepared and used as a cotton impregnant. Imide formation was carried out very carefully at 250-300° F. The product had improved dyeing characteristics over that shown by untreated cloth.

Since certain changes in carrying out the above process, and certain modifications in the product which embody the invention may be made without departing from its scope, it is intended that all matter contained in the foregoing description shall be interpreted as illustrative and not in the limiting sense.

I claim:

1. A process for treating textile fibers which comprises impregnating the fibers with an alkaline aqueous solution of a half-acid amide of a dibasic acid selected from the group consisting of maleic, succinic, glutaric, and phthalic acids, contacting said impregnated fibers with an aqueous solution of a strong mineral acid, and subsequently converting said amide to the corresponding imide by heating said fibers at a temperature within the limits of 200 to 350° F.
2. A process for treating textile fibers which comprises impregnating the fibers with an alkaline aqueous solution of N-hexadecyltetrachlorophthalamic acid, contacting said impregnated fibers with a dilute aqueous solution of a strong mineral acid,

mineral acid, and subsequently heating said fibers to a temperature within the range of 300 to 350° F.

3. A process for treating textile fibers which comprises impregnating the fibers with an alkaline aqueous solution of N-cyclohexylphthalamic acid, contacting said impregnated fibers with a dilute aqueous solution of a strong mineral acid, and subsequently heating said fibers to a temperature within the range of 300 to 350° F.
4. A process for treating textile fibers which comprises impregnating the fibers with an alkaline aqueous solution of N-dodecylphthalamic acid, contacting said impregnated fibers with a dilute aqueous solution of a strong mineral acid, and subsequently heating said fibers to a temperature within the range of 300 to 350° F.
5. A process for treating textile fibers which comprises impregnating such a fiber with an alkaline aqueous solution of a half-acid amide derivative of a primary amine and a di-basic acid capable of forming a cyclic anhydride having from 5 to 6 atoms in the anhydride ring, said half-acid amine containing from 12 to 24 carbon atoms in the molecule, contacting the impregnated fiber with an aqueous solution of a strong mineral acid, and then heating the impregnated fiber at a temperature within the limits of 200 to 350° F.
6. A process for treating textile fibers which comprises impregnating such a fiber with an alkaline aqueous solution of a halogenated half-acid amide derivative of a primary amine and a di-basic acid capable of forming a cyclic anhydride having from 5 to 6 atoms in the anhydride ring, said half-acid amide containing from 12 to 24 carbon atoms in the molecule, contacting the impregnated fiber with an aqueous solution of a strong mineral acid, and then heating the impregnated fiber at a temperature within the limits of 200 to 350° F.
7. A process in accordance with claim 6 wherein said half-acid amide is chlorinated.
8. A textile fiber impregnated with a cyclic imide containing from 12 to 24 carbon atoms in the molecule and having 5 to 6 members in the imide ring.
9. A process for treating textile fibers which comprises impregnating such a fiber with an alkali metal salt of a half-acid amide derivative of a primary amine and a di-basic acid capable of forming a cyclic anhydride having from 5 to 6 atoms in the anhydride ring, said half-acid amide containing from 12 to 24 carbon atoms in the molecule, contacting the impregnated fiber with an aqueous solution of a strong mineral acid, whereby said alkali metal salt is hydrolyzed in situ, and then heating the impregnated fiber at a temperature within the limits of 200 to 350° F., whereby the half-acid amide is dehydrated in situ to form the corresponding imide.
10. A process for treating textile fibers which comprises impregnating such a fiber with an aqueous solution of an alkali metal salt of a half-acid imide derivative of a primary amine and a di-basic acid capable of forming a cyclic anhydride containing from 5 to 6 atoms in the anhydride ring, said half-acid amide containing from 12 to 24 carbon atoms in the molecule, contacting the impregnated fiber with an aqueous solution of a strong mineral acid, whereby said alkali metal salt is hydrolyzed in situ, and then heating the impregnated fiber at a temperature within the limits of 200 to 350° F. for a time within the range of from 1 to 5 minutes, whereby the half-

acid amide is dehydrated in situ to form a corresponding imide.

11. The process of claim 1 wherein said mineral acid is hydrochloric acid.

12. The process of claim 1 wherein said half-acid amide is a derivative of phthalic acid and (trihydroxymethyl) methyl amine.

13. The process of claim 7 wherein said half-acid amine is chlorinated N-dodecyl phthalamic acid.

CHESTER M. HIMEL

#### REFERENCES CITED

The following references are of record in the file of this patent:

#### UNITED STATES PATENTS

| Number    | Name   | Date         |
|-----------|--------|--------------|
| 2,072,770 | Reid   | Mar. 2, 1937 |
| 2,310,873 | Sauer  | Feb. 9, 1943 |
| 2,398,272 | Aelony | Apr. 9, 1946 |

#### Certificate of Correction

Patent No. 2,526,948

October 24, 1950

CHESTER M. HIMEL

It is hereby certified that error appears in the printed specification of the above numbered patent requiring correction as follows:

Column 1, line 10, for "vulnerability" read *vulnerability*; column 3, line 6, for "stage" read *state*; column 4, line 75, for "phthalic" read *phthalamic*; and that the said Letters Patent should be read as corrected above, so that the same may conform to the record of the case in the Patent Office.

Signed and sealed this 16th day of January, A. D. 1951.

[SEAL]

THOMAS F. MURPHY,  
*Assistant Commissioner of Patents.*